

F. CONLIN.  
PROCESS OF FORMING ARMOR PLATE.  
APPLICATION FILED JUNE 25, 1913.

1,186,172.

Patented June 6, 1916.



Witnesses:  
L. Broderick  
J. Frundewall

Frederick Coulia, Inventor  
By his Attorney, Brinsford Wright.

# UNITED STATES PATENT OFFICE.

FREDERICK CONLIN, OF PLAINFIELD, NEW JERSEY.

## PROCESS OF FORMING ARMOR-PLATE.

1,186,172.

Specification of Letters Patent. Patented June 6, 1916.

Application filed June 25, 1913. Serial No. 775,626.

*To all whom it may concern:*

Be it known that I, FREDERICK CONLIN, of Plainfield, in the county of Union, and in the State of New Jersey, have invented a 5 certain new and useful Improvement in Processes of Forming Armor-Plate, and do hereby declare that the following is a full, clear, and exact description thereof.

My invention relates to a process of forming armor plate and has for its object to 10 harden metal by means of a chill at a low cost of manufacture.

Other and further objects of my invention will be apparent from the following description thereof.

For purposes of illustration one manner of carrying out my process is shown in the accompanying drawing, wherein the figure illustrates a section taken through a mold 20 showing the hardening of a body of metal by my process.

In the illustrated embodiment, reference character A indicates a chill of any desired type adapted to abstract heat from, and 25 thereby chill and harden a body of metal cast thereon.

Reference character B indicates a flask or 30 a pit in the foundry floor, adapted to contain sand C in which is formed a mold or cavity D of desired shape. Instead of casting the metal to be hardened directly on chill A, a plate or casting E is placed over the face of the chill, and the metal to be hardened is cast on said plate. In the present embodiment, the plate E preferably is of metal 35 softer and of higher melting point than the metal F cast thereon, as, for example, low-carbon steel such as mild steel or Swedish iron. The metal F cast on said plate E, 40 preferably is of metal harder and of lower melting point than the plate E, as, for example, iron having sufficient carbon to produce these qualities. The face of the chill may be machined or not, and a cope used 45 or not, as conditions require or as may be deemed necessary or advisable.

In operation, the cast metal F is chilled rapidly and hardened by the abstraction of its heat by chill A through plate E, and the 50 heat of the molten cast metal F causes plate E to become sufficiently soft and pasty to tend to cause it to adhere to and unite with casting F. In order to insure a positive union, however, plate E may be provided with projections such as bolts G, 55 which becoming embedded in the cast metal

F, will secure together firmly the two bodies of metal. It is obvious that other securing devices may be used for this purpose.

The completed plate, among other uses, is 60 particularly adapted for use as armor plate, in which case the plate or casting E forms the outer or exposed surface. The body of hardened metal F prevents the penetration of a projectile, and the plate E of comparatively soft metal serves as a deflector or lubricant if the projectile strikes at an angle. If struck squarely by a projectile, the soft metal plate E tends to hold together the body of hardened metal F and prevent it 65 from cracking, shattering, or disintegrating.

It will be understood that the principles above stated may be adapted to special conditions. For example, instead of using a plate E as above described, there could be 70 employed a mild steel casting, particularly in cases where the shape of the completed plate is such as to make it impracticable to form the plate to suit the shape desired, such as curved or rounded plates of conical or 75 other forms.

Many modifications and adaptations of my process will be apparent to those skilled in the art without departing therefrom or from the scope of the claims, the process 80 contemplating the hardening of a body of metal by means of a chill acting through an interposing shield or plate adapted to protect and preserve the chill, and also the casting 85 in connection with a chill of harder metal upon a softer metal.

Having described my invention, what I claim and desire to protect by Letters Patent of the United States is as follows:

1. The process of forming armor plate 90 comprising covering the face of a chill with a layer of metal and pouring a relatively harder metal on said layer of metal.

2. The process of forming armor plate 95 comprising covering the face of a chill with a layer of metal and pouring a relatively higher carbon metal on said layer of metal.

3. The process of forming armor plate 100 comprising covering the face of a chill with a layer of metal and pouring a metal having a relatively lower melting point on said layer of metal.

4. The process of forming armor plate 105 comprising covering the face of a chill with a plate of metal and pouring a relatively harder metal on said plate.

5. The process of forming armor plate

comprising covering the face of a chill with a plate of metal and pouring a relatively higher carbon metal on said plate.

6. The process of forming armor plate 5 comprising covering the face of a chill with a plate of metal and pouring a metal having a relatively lower melting point on said body of metal.

7. The process of forming armor plate 10 comprising covering the face of a chill with a plate of metal and pouring cast iron on said plate.

8. The process of forming armor plate 15 comprising covering the face of a chill with a layer of soft metal and pouring metal on said layer.

9. The process of forming armor plate 20 comprising covering the face of a chill with a layer of low carbon metal and pouring metal on said layer.

10. The process of forming armor plate comprising covering the face of a chill with

a plate of soft metal and pouring metal on said layer.

11. The process of forming armor plate 25 comprising covering the face of a chill with a plate of low carbon metal and pouring metal on said plate.

12. The process of forming armor plate 30 comprising covering the face of a chill with a plate of low carbon steel, securing fastening means in said plate which project therefrom, and pouring cast iron upon said sheet and around said fastening means.

13. The process of forming armor plate 35 by chilling molten metal through an interposing plate of metal having a relatively higher melting point than said molten metal.

In testimony that I claim the foregoing I have hereunto set my hand.

FRED. CONLIN.

Witnesses:

GEORGE L. WODEY,  
E. C. HAND.